

## UNITED STATES PATENT OFFICE

2,513,470

FERROUS ALLOY ARTICLES HAVING GREAT  
STRENGTH AT HIGH TEMPERATURES

Russell Franks and William O. Binder, Niagara Falls, N. Y., assignors, by mesne assignments, to Union Carbide and Carbon Corporation, a corporation of New York

No Drawing. Application May 9, 1946,  
Serial No. 668,332

3 Claims. (Cl. 75—122)

1

This invention relates to ferrous alloy articles for use at high temperatures, referring more particularly to alloy articles suitable for use in applications where great strength at high temperatures is required.

The trend of modern engineering is toward the utilization of high temperatures for many and diverse operations. For example, chemical processes are today conducted at very high temperatures, a notable instance being petroleum refining. Also, the quest for improved power sources has led to the investigation and development of such devices as superchargers, gas turbines, jet propulsion apparatus and the like all operating at high temperatures. These developments demand of the metallurgist metals and alloys which will withstand prolonged exposure to temperatures well above about 700° F. and in many instances well above about 1200° F. The problem is complicated by the fact that severe mechanical stress is often encountered in some metal articles used at these temperatures.

For parts of such devices as superchargers, gas turbines, jet propulsion apparatus and the like, it is necessary to employ alloys that are capable of withstanding severe mechanical stress at high temperatures. Depending upon the design and the intended use of such devices, the temperature ranges at which they operate may be separated into a range between 900° F. and about 1200° F. and into a range upwards of 1200° F. Associated parts and apparatus may be required to withstand temperatures of about 700° F. and above. In devices operating within the lower temperature range, generally much higher stresses are applied than in devices operating above 1200° F. In many instances it is desired that alloys for use in such apparatus be capable of being hot-worked and machined, while in other instances the alloys may be employed in the form of castings. In any event, the alloys must have high strength.

A number of alloys have been proposed for use at high temperatures, but the utility of these alloys has been limited either because they are not hot-workable or machinable or because they become brittle upon prolonged exposure to high temperatures. One of the characteristics of highly alloyed ferrous materials is that as the iron-base solid solution alloy contains more and more of the alloying metals to increase high temperature strength, the stability of the materials at high temperatures tends to decrease so that on prolonged exposure to high temperatures the materials become excessively brittle.

2

It is the principal object of this invention to provide ferrous alloy articles suitable for use in applications where temperatures above about 700° F. are normally encountered. A further object is the provision of hot-workable and machinable alloy articles for use at such elevated temperatures. Another object is the provision of alloy articles capable of withstanding severe mechanical stress at elevated temperatures above about 700° F. A more specific object is the provision of alloys and articles wrought or cast therefrom capable of withstanding severe mechanical stress at elevated temperatures above about 700° F. up to about 1200° F.

In our copending application, Serial No. 599,305, filed June 13, 1945, and matured into Patent No. 2,432,614 of December 16, 1947, we have disclosed alloys which have excellent properties at very high temperatures. The alloys disclosed in that application contain iron, chromium, cobalt, molybdenum, tungsten and at least one element selected from the group consisting of columbium, tantalum, titanium and vanadium.

The present invention comprises heat resisting articles composed of alloys containing 10% to 30% chromium, 10% to 40% cobalt, up to 7.5% molybdenum, 0.5% to 15% tungsten and 0.5% to 3% in the aggregate of at least one metal selected from the group consisting of columbium, tantalum, titanium, and vanadium, the content of any single metal from this group being less than 2%, the remainder of the alloys being nickel and iron except for incidental impurities and small quantities of elements customarily present in steels of good quality. The iron content of the alloys of the present invention should be at least 10% and the nickel content should be less than 15%. The tungsten content should be not less than 7.5% in the absence of molybdenum. A generally preferred range for molybdenum, if molybdenum is present, is 0.5% to 5%.

Carbon is always present in the alloys of the invention. Preferably it does not exceed about 1%, and if hot working of the alloys is desired, the maximum carbon content should be 0.35%. Nitrogen is importantly beneficial and should be present in a proportion of 0.05% to 0.25%. Silicon and manganese may be present, the silicon content preferably not exceeding 1% and the manganese content not exceeding 2% if hot working is desired.

A useful test for determining the suitability of materials for use at high temperatures is the so-called stress-rupture test. In this test several samples of an alloy to be tested are maintained

at a given temperature, each sample being subjected to a different measured stress. The time required to cause failure of the samples under these conditions of temperature and stress is determined, and the time and stress values obtained are plotted to yield a curve for the particular material under test. From this curve can be determined the stress the material will withstand for a given period of time, say 1000 hours, at the particular temperature for which the curve was drawn. This test provides a convenient method of determining the load carrying ability of a material. It also gives some indication of whether or not the material becomes embrittled upon prolonged exposure at the temperature of the test. A brittle material will break without elongation, whereas ductile material will elongate before failure.

Stress-rupture tests conducted in the manner just described indicate that the alloys of the invention maintain great strength at temperatures as high as 1500° F. and that even at such high temperature the alloys possess good ductility.

Typical examples of the high temperature strength of alloys within the invention are set forth in the table below. In this table are reported the result of stress-rupture tests in which a stress of 20,000 pounds per square inch was applied to several samples of the alloys to be tested while the samples were maintained at a temperature of 1500° F. The time in hours required for the sample to fail under these extremely severe conditions is reported in the table. Some of the samples were in the as-forged condition (condition 1), others had been forged, heated one hour at 1250° C. and quenched in water (condition 2).

Table

| Composition—Remainder Substantially all Fe |                   |                   |                   |                  |                   |                  |                  | Hours to Fail<br>@ 1500° F. and<br>20,000 p. s. i.<br>stress: Condi-<br>tion |     |
|--------------------------------------------|-------------------|-------------------|-------------------|------------------|-------------------|------------------|------------------|------------------------------------------------------------------------------|-----|
| Per<br>Cent<br>Cr                          | Per<br>Cent<br>Ni | Per<br>Cent<br>Co | Per<br>Cent<br>Mo | Per<br>Cent<br>W | Per<br>Cent<br>Cb | Per<br>Cent<br>C | Per<br>Cent<br>N | 1                                                                            | 2   |
| 18                                         | 10                | 30                | 3                 | 2                | 1                 | 0.15             | 0.12             | 117                                                                          | 143 |
| 18                                         | 10                | 30                | 3                 | 10               | 1                 | 0.15             | 0.12             | 48                                                                           | 182 |
| 18                                         | 10                | 30                | 0.5               | 15               | 1                 | 0.15             | 0.12             | 34                                                                           | 251 |

The data in the above table clearly illustrate the ability of the alloys of the invention to withstand large stresses at elevated temperatures for prolonged periods of time without failure.

In manufacturing the alloys of this invention care should be taken that the composition limits set forth be closely adhered to with regard to the intended use of the alloys since material variations in the proportions of the several ingredients detrimentally affect the desired properties. For example, if the alloys are to be employed as castings, the carbon content may be as high as 1%; but if hot-workability is desired, the carbon content should be kept at a maximum of about 0.35% and preferably should not exceed 0.2%.

Similarly, the proportions of molybdenum, tungsten, columbium, tantalum, titanium and vanadium present in the alloys affect hot-workability and weldability. Too high a proportion of any of these elements has a detrimental effect on hot-workability and weldability, particularly the latter property. Alloys within the composition limits defined may be welded readily by any of the common welding methods, for example, electric arc, oxyacetylene, submerged-melt electric welding, or solid phase pressure welding,

sound, strong and tough welds being produced without undue embrittlement of weld metal or base metal, and such welds retain their toughness at elevated temperatures. However, if too high a proportion of any of these elements is present in the alloys, welds produced usually suffer from loss of toughness at elevated temperatures.

The presence of nitrogen in the alloys of the invention within the range indicated is important, nitrogen having a beneficial effect on the high temperature stability of the alloys.

The alloys of the invention are preferably worked in the range 2100° F. to 1600° F. In some cases working may be continued to a temperature somewhat below the recrystallization temperature (about 1200° F.). Alloys so wrought are said to be in the "cold hot-worked" condition. They may be used in this condition in applications where temperatures not above 1200° F. are encountered. For use at temperatures much above 1200° F., the alloys of the invention should be annealed at about 2200° F. to 2320° F. before use.

Being hot-workable, machinable, weldable, and castable, and possessing remarkable strength at elevated temperatures up to about 1200° F., the alloys of the invention are particularly well suited to use in the fabrication of articles such as parts of superchargers, gas turbines, jet propulsion apparatus and the like which are required to withstand severe mechanical stress at elevated temperatures. Their freedom from embrittlement upon prolonged exposure at high temperatures recommends their use where dependability of operation is essential.

This application is a continuation-in-part of

50 our copending application, Serial No. 599,305, filed June 13, 1945, now Patent No. 2,432,614, issued December 16, 1947.

We claim:

1. A heat resisting ferrous alloy article capable of withstanding severe mechanical stress at elevated temperatures above 700° F. for prolonged periods of time and having high strength and stability at such elevated temperatures, said article being composed of a machinable, weldable, castable and hot-workable ferrous alloy consisting of 10% to 30% chromium; 10% to 40% cobalt; 0% to 7.5% molybdenum; 0.5% to 15% tungsten but not less than 7.5% tungsten in the absence of molybdenum; 0.5% to 3% in the aggregate of at least one metal selected from the group consisting of columbium, tantalum, titanium and vanadium, the amount of any single metal selected from this last named group being less than 2%; carbon in an amount not exceeding 0.35%; 0.05% to 0.25% nitrogen; silicon in an amount not exceeding 1%; manganese in an amount not exceeding 2%; the remainder of said alloy consisting of nickel and iron except for 55 incidental impurities such nickel content being

present in an amount less than 15% and such iron content being at least 10%.

2. A heat resisting ferrous alloy article capable of withstanding severe stresses when used at elevated temperatures upwards of 700° F. for prolonged periods of time as herein set forth, said article being composed of a machinable, weldable, castable and hot-workable ferrous alloy consisting of 10% to 30% chromium; 10% to 40% cobalt; 0% to 7.5% molybdenum; 0.5% to 15% tungsten but not less than 7.5% tungsten in the absence of molybdenum; 0.5% to less than 2% columbium; 0.05% to 0.25% nitrogen; carbon in an amount not exceeding 0.35%; silicon in an amount not exceeding 1%; manganese in an amount not exceeding 2%; the remainder of said alloy consisting of nickel and iron except for incidental impurities such nickel content being present in an amount less than 15% and such iron content being at least 10%.

3. A heat resisting ferrous alloy article capable of withstanding stresses of the order of 20,000 p. s. i. when used at elevated temperatures of the order of 1500° F. for prolonged periods of times as herein set forth, said article being composed of a machinable, weldable, castable and hot-workable ferrous alloy consisting substantially of 18% chromium; 30% cobalt; 0.5% molybdenum; 15% tungsten; 1% columbium; 0.15% carbon; 0.12% nitrogen; the remainder of said alloy consisting of nickel and iron except for incidental impurities such nickel content being 10% and such iron content being at least 10%.

RUSSELL FRANKS.

WILLIAM O. BINDER.

20 25 30

The following references are of record in the file of this patent:

#### UNITED STATES PATENTS

| Number    | Name          | Date           |
|-----------|---------------|----------------|
| 1,376,062 | Albrecht      | Apr. 26, 1921  |
| 1,729,154 | Clawson       | Sept. 24, 1929 |
| 1,774,862 | Wissler       | Sept. 2, 1930  |
| 2,213,207 | De Golyer     | Sept. 3, 1940  |
| 2,244,517 | De Golyer     | June 3, 1941   |
| 2,245,366 | Rohn          | June 10, 1941  |
| 2,309,372 | Wissler       | Jan. 26, 1943  |
| 2,397,034 | Mohling       | Mar. 19, 1946  |
| 2,398,702 | Fleischmann   | Apr. 16, 1946  |
| 2,432,614 | Franks et al. | Dec. 16, 1947  |
| 2,432,615 | Franks et al. | Dec. 16, 1947  |
| 2,432,618 | Franks et al. | Dec. 16, 1947  |

#### FOREIGN PATENTS

| Number  | Country       | Date          |
|---------|---------------|---------------|
| 219,293 | Great Britain | May 7, 1925   |
| 308,549 | Great Britain | Mar. 28, 1929 |

#### OTHER REFERENCES

- 25 Kinzel and Franks: Alloys of Iron and Chromium, published by McGraw-Hill Book Co., N. Y., vol. II. 1940, pages 87, 88, 180, 192, 194, 455.
- 30 Progress Report on NDRC, Research Project NRC-8, P. B. 39, 578, October 7, 1942, pages 1-21 inclusive (particularly page 5). Declassified to open January 28, 1946.